

## UNITED STATES PATENT OFFICE

2,304,874

## LUBRICANT

Edward R. Barnard, Chicago, Ill., assignor to  
Standard Oil Company, Chicago, Ill., a corpora-  
tion of Indiana

No Drawing. Application September 26, 1940,  
Serial No. 358,429

5 Claims. (Cl. 252—53)

This invention relates to improvements in lub-  
ricants and particularly to lubricants of the type  
of motor oils.

It is an object of the present invention to pro-  
vide an improved motor oil having favorable tem-  
perature viscosity characteristics and greatly im-  
proved engine wear properties.

It is a further object of the invention to pro-  
vide a motor oil having favorable stability, min-  
imum resin, varnish and/or carbon formation.

A still further object of the invention is to pro-  
vide a motor oil having, in addition to the fore-  
going advantages, excellent consumption charac-  
teristics.

I have discovered that a motor oil providing  
the above desired characteristics can be obtained  
by blending a narrow cut mineral lubricating oil,  
preferably a narrow cut solvent extracted mineral  
lubricating oil, and a synthetic lubricating oil of  
the type hereinafter described.

The narrow cut mineral lubricating oil is pref-  
erably a raffinate of a solvent extracted mixed  
base petroleum distillate which is distilled to pro-  
duce a relatively narrow cut fraction. The raf-  
finate may be obtained by any of the well-known  
solvent extraction processes, such as the furfural  
process, the phenol process, the sulfur dioxide  
process, the sulfur dioxide-benzol process, the  
nitro benzene process, the nitro benzene-sulfuric  
acid process or the Chlorex process.

In preparing the motor oils of the various  
grades it is the usual practice to prepare base oils  
of the 20 S. A. E. grade and of the 50 S. A. E.  
grade which are then blended in the proper pro-  
portions to produce intermediate grades of oils.  
In preparing the base oils in accordance with the  
present invention the solvent extracted distillate  
is distilled, preferably under reduced pressure, to  
remove both the light ends and the heavier ends  
of the fraction, the distillation being carried out  
so that the initial boiling point under 1 milli-  
meter mercury pressure is at least about 400° F.  
and the difference in temperature between the  
initial distillation temperature at 1 millimeter  
mercury pressure and the temperature at which  
90% distills under 1 millimeter mercury pressure  
is not greater than about 200° F. and preferably  
not greater than about 185° F. The term "nar-  
row cut" as used herein and in the appended  
claims refers to distillates in which the differ-  
ence between the initial distillation temperature  
and the distillation temperature at the 90%  
point, both at 1 millimeter mercury pressure is  
not greater than about 200° F. The 90% distil-  
lation temperature referred to herein is a meas-  
ure of the tendency of lubricating oils to form  
carbon in internal combustion engines, and is  
determined by distilling a 200 cubic centimeter  
sample of the oil at 1 millimeter mercury pres-  
sure and determining the temperature of the  
vapor when 90% has distilled. The test is de-  
scribed in detail by W. H. Bahlike et al. in the  
S. A. E. Journal, vol. 29, 1931 (page 215). This  
90% distillation point is also referred to as the  
Carbonization Index of the oil.

The elimination of the lighter and less volatile  
components of the raffinate oil effects a consider-  
able improvement in oil consumption while the  
removal of heavier fractions from the raffinate  
reduces the combustion chamber carbon forma-  
tion to a large degree, and furthermore, such  
carbon as is formed by a narrow cut raffinate oil  
is softer and more easily removed and is thus less  
liable to cause scratching of the piston rings,  
cylinder bores and the like of the engine.

Illustrative of suitable base oils of the im-  
proved motor oils prepared in accordance with  
the present invention are the 20 S. A. E. and the  
50 S. A. E. oils having the following inspections:

|                                                    | 20 SAE  | 50 SAE  |
|----------------------------------------------------|---------|---------|
| Gravity, °A. P. I.                                 | 28.3    | 26.8    |
| Flash, °F.                                         | 415     | 510     |
| Pour point, °F.                                    | -5      | +10     |
| Saybolt viscosity at 100° F.                       | seconds | seconds |
| Saybolt viscosity at 210° F.                       | seconds | seconds |
| Viscosity index                                    | 56.4    | 103     |
| Carbonization index, °F.                           | 93      | 85      |
| Initial distillation temperature, °F. <sup>1</sup> | 535     | 640     |
|                                                    | 400     | 470     |

<sup>1</sup> At 1 m. m. of mercury absolute pressure.

The above oils are raffinates of Chlorex ex-  
tracted distillates of a Mid-Continent crude oil.

The synthetic lubricating oil is preferably one  
obtained by polymerizing, in the liquid phase, an  
iso-mono-olefin such as isobutylene or a hydro-  
carbon mixture containing the same at a tem-  
perature of from about 0° F. to about 100° F.  
preferably at 32° F. in the presence of a catalyst  
such as boron fluoride, aluminum chloride, zinc  
chloride or other similar active halide catalyst  
of the type employed in the Friedel-Crafts reac-  
tion. I may also employ the co-polymers of iso-  
mono-olefins with normal olefins. In the prepara-  
tion of the polymers I may employ, for exam-  
ple, liquid isobutylene or a hydrocarbon mixture  
containing the same such as a butane-butylene  
fraction recovered from petroleum gases, espe-  
cially those gases produced in the cracking of  
petroleum oils for the manufacture of gasoline.  
This light fraction may contain from about 10%

to about 25% isobutylene, the remainder being principally butenes and normal butane. The hydrocarbon mixture containing 10% to 25% isobutylene is maintained under pressure sufficient to keep it in the liquid phase and cooled by suitable means to a temperature of for example, about 32° F. and from about 1% to about 2% boron fluoride based upon the isobutylene content of the material treated added with vigorous agitation. Excessive rise in temperature due to the heat of the reaction may be avoided by efficient cooling. After the polymerization of the isobutylene, together with a relatively minor amount of the normal olefins present, the reaction mass is neutralized and washed free of the acidic substances arising from the catalysts, the acidic substances arising from the catalysts, the oily layer separated, and the polymer subsequently segregated from the unreacted hydrocarbons by distillation. The polymer mixture so obtained depending upon the temperature of the reaction varies in consistency from a light liquid to a viscous oil-like material and contains polymers having molecular weights ranging from about 100 to 1500. The polymer so obtained is then vacuum distilled to remove the lighter and heavier fractions therefrom and to produce a final product having a Saybolt viscosity at 210° F. of about 185 seconds to 500 seconds and a flash point of about 350° F. to about 440° F.

In accordance with the present invention an improved motor oil is obtained by blending a narrow cut raffinate oil with from about 1% to about 40% and preferably from about 3% to about 20% of an olefin polymer of the type described. To the blend I may add a small amount, 0.05% to 0.5%, of an anti-wear agent such as tributyl phosphite, diethyl sulfone, triethyl phosphate, methyl dichloro stearate, etc. Blends of this composition show improved resistance to oxidation, substantially reduce varnish formation in internal combustion engines, and markedly reduce engine wear.

In the following tables are presented data of various tests employing blends of a narrow cut raffinate oil and various concentrations of an isobutylene polymer. The control oil in each of these tests is a narrow cut raffinate having the following specifications:

|                                                                 |                  |      |
|-----------------------------------------------------------------|------------------|------|
| Gravity                                                         | degrees A. P. I. | 28.3 |
| Flash                                                           | degrees F.       | 415  |
| Pour point                                                      | do               | -5   |
| Saybolt viscosity at 100° F.                                    | seconds          | 382  |
| Saybolt viscosity at 210° F.                                    | do               | 56.4 |
| Viscosity index                                                 |                  | 93   |
| Carbonization index                                             | degrees F.       | 535  |
| Initial boiling point (at 1 m. m. of mercury absolute pressure) | degrees F.       | 400  |

The isobutylene polymer used in the blends had the following characteristics:

|                              |                  |      |
|------------------------------|------------------|------|
| Gravity                      | degrees A. P. I. | 32.7 |
| Flash                        | degrees F.       | 365  |
| Pour point                   | do               | -35  |
| Saybolt viscosity at 100°    | seconds          | 469  |
| Saybolt viscosity at 210° F. | do               | 58   |
| Viscosity index              |                  | 75   |
| Carbonization index          | degrees F.       | 470  |

The sludging time data of various blends of narrow cut raffinate oil and isobutylene polymers are tabulated in Table I. The sludging time is the number of hours required for the samples to form 10 milligrams and 100 milligrams of sludge when maintained at a temperature of

about 341° F. while air is being bubbled therethrough.

Table I

| Sample                             | Sludging time (hrs.) |                 |
|------------------------------------|----------------------|-----------------|
|                                    | 10 milli-grams       | 100 milli-grams |
| (1) Control (narrow cut raffinate) | 83                   | 140             |
| (2) (1)+3% isobutylene polymer     | 100                  | 166             |
| (3) (1)+5% isobutylene polymer     | 110                  | 176             |
| (4) (1)+10% isobutylene polymer    | 180                  | 210             |
| (5) (1)+15% isobutylene polymer    | 200-240              | 200-240         |
| (6) (1)+20% isobutylene polymer    | 300+                 | 300+            |
| (7) (1)+50% isobutylene polymer    | 300+                 | 300+            |

The above data show that increasing the concentration of isobutylene polymer produces an increase in the sludging time.

In motor oils it is highly desirable that there be a minimum increase in the viscosity of the oil as the oxidation of the oil proceeds, in other words, there should be a minimum increase in the viscosity of the oil during use. The effect upon the viscosity increase of blends of a narrow cut raffinate oil and an isobutylene polymer upon oxidation at 341° F. in the presence of air is shown by the data presented in Table II. Also in Table II, in parenthesis, are tabulated the viscosity indices of the control oil and the blends for the corresponding oxidation periods. The viscosity indices in Table II are determined by the Dean and Davis method described in the Oil and Gas Journal of March 31, 1932, page 92.

Table II

| Sample                             | Saybolt viscosity at 100° F. (seconds) after oxidation at 341° F. for— |            |            |
|------------------------------------|------------------------------------------------------------------------|------------|------------|
|                                    | 0 hrs.                                                                 | 48 hrs.    | 96 hrs.    |
| (1) Control (narrow cut raffinate) | 372 (94.2)                                                             | 409 (92.5) | 540 (77.2) |
| (2) (1)+3% isobutylene polymer     | 376 (92.8)                                                             | 415 (92.4) | 527 (71.5) |
| (3) (1)+5% isobutylene polymer     | 377 (92.5)                                                             | 415 (92.4) | 536 (86. ) |
| (4) (1)+10% isobutylene polymer    | 381 (91.0)                                                             | 419 (90.0) | 497 (89.2) |
| (5) (1)+15% isobutylene polymer    | 383 (90.3)                                                             | 420 (93.0) | 502 (94.3) |
| (6) (1)+20% isobutylene polymer    | 381 (91.0)                                                             | 444 (84.0) | 489 (90.5) |
| (7) (1)+50% isobutylene polymer    | 403 (85. )                                                             |            | 707 (81. ) |

Blends containing more than 50% of isobutylene polymer show a marked decrease in the viscosity index, whereas blends containing less than 50% of the polymer show little change in the viscosity index. It will be observed that after 96 hours of oxidation the control oil showed a substantial decrease in the viscosity index, but blends of from about 10% to about 40% of the polymer showed only a very slight decrease in the viscosity index after oxidation for an equivalent period.

If desired other addition agents, such as pour point depressors, antioxidants, sludge dispersers and the like may be added, without departing from the scope of the present invention as defined by the appended claims.

I claim:

1. An improved lubricant comprising a narrow cut solvent extracted petroleum oil having a 90% distillation point under 1 millimeter mercury pressure not substantially greater than about 200° F. above the initial boiling point at 1 millimeter mercury pressure, and from about 1% to about 40% of an isobutylene polymer having a

Saybolt viscosity at 210° F. of about 185 seconds to about 500 seconds and a flash point of about 350° F. to about 450° F.

2. An improved motor oil comprising a solvent extracted petroleum oil having a 90% distillation point under 1 millimeter mercury pressure not substantially greater than about 200° F. above the initial boiling point at 1 millimeter mercury pressure and from about 3% to about 20% of an isobutylene polymer having a Saybolt viscosity at 210° F. of from about 185 seconds to about 500 seconds.

3. An improved motor oil which is substantially resistant to oxidation, substantially non-varnish forming, and which has low consumption and carbon forming characteristics comprising a narrow cut solvent extracted petroleum oil having a 90% distillation point under 1 millimeter mercury pressure not greater than about 200° F.

above the initial boiling point at said pressure, from about 1% to about 40% of an isobutylene polymer having a Saybolt viscosity at 210° F. of about 185 seconds to about 500 seconds and a small amount of an anti-wear agent.

4. An improved motor oil as described in claim 3 in which the anti-wear agent is tributyl phosphite.

5. An improved lubricant comprising a narrow cut solvent extracted petroleum oil having a 90% distillation point under 1 millimeter mercury pressure not substantially greater than about 200° F. above the initial boiling point at 1 millimeter mercury pressure, and from about 1% to about 40% of an iso-mono-olefin polymer having a Saybolt viscosity at 210° F. of about 185 seconds to about 500 seconds and a flash point of about 350° F. to about 450° F.

EDWARD R. BARNARD.